

Patented Jan. 8, 1929.

1,698,660

# UNITED STATES PATENT OFFICE.

HUGH T. STEWART, OF NEW YORK, N. Y., ASSIGNOR TO METALASTIC INC., OF JERSEY CITY, NEW JERSEY, A CORPORATION OF NEW JERSEY.

## PACKING.

No Drawing.

Application filed July 26, 1922. Serial No. 577,761.

This invention relates to packing such as may be used in various mechanical devices for the purpose of sealing joints or connections between parts which may or may not 5 have relative movement.

An object of the invention is to provide an improved packing which when used between relatively moving parts offers a minimum resistance to relative movement, which is self 10 lubricating, which can be fitted to any size or shape of cavity, which will not harden, which will withstand high temperatures and pressures, which may be used without cutting or shaping, and with which wear of the 15 relatively moving parts is reduced to a minimum.

A further object is to provide an improved packing for accomplishing each and all of the above objects, having low heat conductivity, which is elastic and plastic, and which 20 is relatively inexpensive. Other objects and advantages will be apparent from the following description of a practical form of the invention and the novel features will be 25 pointed out in claims.

The packing comprises lubricating oil, asbestos fibre, graphite, and babbitt or other suitable anti-friction metal or alloy. Any suitable lubricating oil may be used but it 30 should preferably have a viscosity of not less than 30.0 and not more than 80.0 (Engler) at 50° C. and not more than 5.0 and less than 1.0 at 180° C. The specific gravity at 15° C. should not be less than .500 or more than .980 in order to obtain the best results. The flash point should also preferably be above 200° C. and less than 350° C. in an open pan test. It has been found that the standard A. C. transformer oil is a very satisfactory product for the oil component of the 40 improved packing.

The asbestos fibre should be in the form of shreds, preferably varying from about 3 mm. in length and 0.25 mm. in diameter to 45 about 7 mm. in length and 1.5 mm. in diameter.

The graphite, which forms a solid lubricant, should be finely divided or comminuted, preferably in the form of flakes not larger than about 2 mm. in diameter and 0.05 mm. in thickness. It has been found that Dixon #2 graphite proves very satisfactory as the graphite component of the packing.

The metal or alloy component of the packing should be finely divided, such as in the

forms of chips preferably not larger than 5 mm. in length, 3 mm. in width, and 0.5 mm. in thickness, and diminishing to pulverized form. The slightly rough edges of the metallic chips enable the asbestos to hold the 60 chips in position. By the term "chips" I mean a form of particles which may be readily obtained from commercial Babbitt metal, as distinguished from particles which must be specially formed. The chips are obtained 65 by the action of a suitable cutting tool upon a piece of commercial Babbitt metal and the result is that the chips are formed with sharp edges which, when the chips are mixed with the fibre, will help to shred the fibre. 70

The preferred proportions in which the components are mixed are as follows, the portions being given by weight:

|          | Parts. |
|----------|--------|
| Asbestos | 14 75  |
| Oil      | 7      |
| Metal    | 68     |
| Graphite | 11     |

Any suitable metal or alloy may be used, 80 but should preferably be babbitt, lead, or similar metals or alloys. A very satisfactory anti-friction alloy for this purpose is the following:

Tin 83.75% to 84.25%, copper 6.75%, anti- 85 mony 8.75% to 9.25%, iron not over .02%, lead not over .02%.

Any of the usual Babbitt metals may also be used.

In the preferred preparation of the mixture, the carded asbestos fibre and oil are mixed and heated to about 100° C., after which the babbitt is added and mixed, then the graphite. The temperature should always be less than the fusion temperature of 95 the metal or alloy. After the component materials have been thoroughly mixed they may be cooled, and the mixture is then ready for use. It has plasticity such that it can be packed into any desired shape or size of cavity. There is enough elasticity when molded and compressed to cause it to fit closely to the packed parts with an even pressure and maintain the close fit for an extended period.

The graphite and oil form a superior lubricant for moving parts and the capillary action of the small particles draws oil continuously to the bearing surfaces. The oil also prevents caking of the graphite. The asbestos, which is of itself of such a nature as 100 105 110

to withstand such chemical action as might take place within the composition, binds together the various particles, and prevents action of heat upon the body of oil in the packing. The entire packing is loose non-combustible and can be added to a cavity little by little without waste. The packing is convenient, efficient, durable, easily and quickly applied and relatively inexpensive. When removed from a stuffing box it may be easily pulled apart and returned to its original loose condition.

It will be understood that the proportions given herein are those which have been found to be the most satisfactory and that this is for the purpose of explaining the nature of the invention. Obviously various minor changes in proportions and equivalents of the component parts or the manner of mixing may be made by those skilled in the art within the principle and scope of the invention.

I claim:

1. A stuffing box packing material comprising an intermixture of small chips of babbitt, comminuted graphite, asbestos fibres, and lubricating oil which has been heated to a temperature of approximately 100° C. and less than the temperature at which the babbitt fuses.
2. A stuffing box packing material comprising an intermixture of approximately 68 parts of small chips of babbitt, 11 parts of comminuted graphite, 14 parts of asbestos fibres, and 7 parts of lubricating oil, the proportions being by weight.
3. A stuffing box packing material comprising an intermixture of babbitt chips, graphite, asbestos fibres and lubricating oil in such minor proportions that the resulting mass is loose in texture.
4. A stuffing box packing material comprising an intermixture of babbitt chips,

flake graphite, asbestos fibres and A. C. standard transformer oil.

5. The method of preparing a packing material which comprises heating asbestos fibres and oil to approximately 100° C. then adding babbitt chips and comminuted graphite and mixing.

6. The method of preparing a packing material which comprises mixing fibre and oil, adding particles of anti-friction metal and mixing again, and then adding a solid lubricant and mixing again.

7. The method of preparing a packing material which comprises mixing fibre and oil, heating the mixture to about 100° C., adding particles of anti-friction metal and mixing again, and then adding a solid lubricant and mixing again.

8. The method of preparing a packing material which comprises mixing fibre and oil, heating the mixture to about 100° C., adding particles of anti-friction metal and mixing again, then adding a solid lubricant and mixing again, and maintaining the temperature throughout at less than the fusion temperature of the metal.

9. A loose packing material comprising a mixture of chips of anti-friction metallic material, fibre, graphite, and oil in such minor proportions that the resulting mass is loose in texture.

10. A stuffing box packing material comprising an intermixture of small chips of babbitt, comminuted graphite, asbestos fibers, and lubricating oil which has been preheated to a temperature less than a temperature at which the babbitt fuses in such minor proportions that the resulting mass is loose in texture.

In testimony whereof I have hereunto set my hand.

HUGH T. STEWART.